



US005865953A

**United States Patent** [19]**Rottger et al.****Patent Number:** **5,865,953****Date of Patent:** **Feb. 2, 1999**[54] **PAPER FOR CORRUGATING MEDIUM**[75] Inventors: **Mark A. Rottger**, Westford; **Mark R. Leonard**, Southborough, both of Mass.[73] Assignee: **Merrimac Paper Company, Inc.**, Lawrence, Mass.[21] Appl. No.: **706,343**[22] Filed: **Aug. 30, 1996**[51] **Int. Cl.<sup>6</sup>** ..... **D21F 11/00**; D21H 17/60[52] **U.S. Cl.** ..... **162/184**; 162/135; 162/158;  
162/172; 162/164.1[58] **Field of Search** ..... 162/184, 135,  
162/169, 158, 164.3, 164.1, 172, 173[56] **References Cited**

## U.S. PATENT DOCUMENTS

|           |         |                  |       |           |
|-----------|---------|------------------|-------|-----------|
| 2,229,620 | 1/1941  | Bradner          | ..... | 162/184   |
| 2,993,800 | 7/1961  | Pickell          | ..... | 162/172   |
| 3,033,708 | 5/1962  | McKee            | ..... | 117/119.8 |
| 3,109,769 | 11/1963 | Martin           | ..... | 162/164   |
| 3,119,731 | 1/1964  | Ströle et al.    | ..... | 162/164   |
| 3,173,829 | 3/1965  | Thier et al.     | ..... | 162/141   |
| 3,250,666 | 5/1966  | Clark et al.     | ..... | 162/169   |
| 3,298,902 | 1/1967  | Osborg et al.    | ..... | 162/158   |
| 3,307,994 | 3/1967  | Scott, Jr.       | ..... | 156/210   |
| 3,308,006 | 3/1967  | Kresse et al.    | ..... | 161/137   |
| 3,518,216 | 6/1970  | Harvey et al.    | ..... | 260/28.5  |
| 3,525,668 | 8/1970  | Goldstein        | ..... | 162/169   |
| 3,659,772 | 5/1972  | Dorsey et al.    | ..... | 229/3.1   |
| 3,687,767 | 8/1972  | Reisman et al.   | ..... | 156/210   |
| 3,849,224 | 11/1974 | Hintz et al.     | ..... | 156/208   |
| 3,920,496 | 11/1975 | Wilkinson et al. | ..... | 156/82    |
| 4,038,122 | 7/1977  | DeLigt           | ..... | 156/210   |
| 4,054,717 | 10/1977 | Gill et al.      | ..... | 428/452   |
| 4,086,116 | 4/1978  | Yazaki et al.    | ..... | 156/205   |
| 4,409,274 | 10/1983 | Chaplin et al.   | ..... | 428/112   |

|           |         |                |       |         |
|-----------|---------|----------------|-------|---------|
| 4,567,215 | 1/1986  | Jackson et al. | ..... | 523/218 |
| 4,609,431 | 9/1986  | Grose et al.   | ..... | 162/135 |
| 5,152,872 | 10/1992 | Racine et al.  | ..... | 162/184 |
| 5,242,545 | 9/1993  | Bradway et al. | ..... | 162/135 |
| 5,292,391 | 3/1994  | Wallck         | ..... | 156/205 |

## FOREIGN PATENT DOCUMENTS

450523 8/1948 Canada ..... 162/172

## OTHER PUBLICATIONS

George L. Booth "Coating equipment and Processes", Lockwood Publishing Co., Inc. pp. 158-162 and 452-453, Jan. 1970.

Kellicutt et al., "strength evaluations of corrugated containers by the drop test method", TAPPI, vol. 39, No. 9, pp. 62A-70A, Sep. 1956.

Trosset et al., "A study of some factors which affect the stiffness of folding boxboard", TAPPI, vol. 41, No. 3, pp. 177A-186A, Mar. 1958.

Krasniewski, Jr., J., "Paper Coating Additives", *Tappi Press*, 1995, p. 74.*Primary Examiner*—Stanley S. Silverman*Assistant Examiner*—José A. Fortuna*Attorney, Agent, or Firm*—Foley, Hoag & Eliot LLP

[57]

## ABSTRACT

Making paper for corrugating medium includes forming a sheet of pulp material, partially drying the sheet of pulp material to provide a partially dried sheet, applying a crack-reducing agent to surfaces of the partially dried sheet, and providing a sheet of paper by drying the partially dried sheet after applying the crack-reducing agent. Forming a sheet of pulp material may include providing a pulp slurry to a headbox having a slice and carrying the pulp slurry that exits from the slice away from the headbox using, for example, a Fourdrinier. The Fourdrinier may also dry the sheet.

15 Claims, 4 Drawing Sheets





FIG. 1



FIG. 2A



FIG. 2B



FIG. 3



FIG. 4



FIG. 5

## PAPER FOR CORRUGATING MEDIUM

## TECHNICAL FIELD

This application relates to the field of making paper and more particularly to the field of making paper that is used for corrugating medium.

## BACKGROUND OF THE INVENTION

Corrugated board is made by attaching one or more flat sheets of paper to a medium, a wavy or fluted section of paper. The medium may be formed using any one of a variety of conventional and well-known corrugation processes that provide any one of a variety of flute sizes. In applications that call for relatively small flute sizes, corrugating the medium sometimes results in cracks forming in the paper. In addition, when only one flat sheet is attached to the medium, such as in the case of certain types of gift boxes, then the cracks become visible and aesthetically unappealing. Many solutions to this problem have been suggested in the prior art, as described below.

U.S. Pat. No. 3,687,767 to Reisman et al. discloses preventing cracks in corrugating medium by first treating the paper with a resin and then drying the resin. The paper is then corrugated and, following that, is heat treated to cure the resin. This curing step is shown in the flow chart of FIG. 1 of Reisman et al. in the fourth step from the bottom. Similarly, U.S. Pat. No. 3,173,829 to Thier et al. is directed to a process in which an additive is provided to the paper pulp prior to the sheet forming and drying process. After the paper has been manufactured, the additive (bonding agent) is activated by heat and/or pressure.

Both the Reisman et al. and Thier et al. schemes require an extra curing or activating step after the paper has been manufactured. This may be impractical in some situation such as, for example, a large corrugated board manufacturing operation that is not readily equipped to incorporate this extra step into their process. In addition, in cases where curing or activation is provided by heat, an inadvertent and premature exposure of the product to heat may cause undesirable results.

U.S. Pat. No. 3,033,708 to McKee, U.S. Pat. No. 3,307,994 to Scott, Jr., U.S. Pat. No. 3,308,006 to Kresse et al., U.S. Pat. No. 3,518,216 to Harvey et al., U.S. Pat. No. 3,659,772 to Dorsey et al., and U.S. Pat. No. 4,038,122 to DeLigt are all directed to applying an additive to the finished paper product during, or just prior to, corrugation in order to prevent cracks during the corrugation process. However, applying the additive to the finished paper product adds another step and requires extra machinery located either at the corrugator or at the paper manufacturer. In addition, applying an additive to the finished paper product can create difficulties with respect to handling any excess additive that does not adhere to the paper.

U.S. Pat. No. 3,109,769 to Martin, U.S. Pat. No. 3,119,731 to Strole et al., U.S. Pat. No. 3,298,902 to Osborg et al., and U.S. Pat. No. 3,525,668 to Goldstein et al. all appear to be directed to providing an additive to the pulp during the paper manufacturing process. Although this arguably avoids the need for extra equipment to apply the additive, it does result in a relatively large amount of additive being used since the additive ends up being applied throughout the entirety of the paper, rather than just at the surfaces.

In chapter 7 of a 1995 textbook titled "Paper Coating Additives" published by Tappi Press of Atlanta, Ga., the author suggests that dilutions of oxidized polyethylene

emulsions have been applied at a size press or through surface spraying to lower surface coefficient of friction. The author goes on to state that spraying the oxidized polyethylene emulsions in the manufacture of corrugating medium decreases cracking during the corrugation step. However, since the author suggests only spraying to reduce cracking (as opposed to applying the emulsion with a size press to improve the coefficient of friction), this solution is similar to the solutions in references discussed above that disclose applying an additive after the paper manufacturing process is complete or just prior to corrugation.

It is desirable, therefore, to prevent cracks in the corrugated bound medium in an economical and feasible manner.

## SUMMARY OF THE INVENTION

According to the present invention, making paper for a corrugating medium includes forming a sheet of pulp material, partially drying the sheet of pulp material to provide a partially dried sheet, applying a crack-reducing agent to surfaces of the partially dried sheet, and providing a sheet of paper by drying the partially dried sheet after applying the crack-reducing agent. The partially dry sheet may contain between 1% and 25% (by weight) moisture and, in a preferred embodiment, the partially dry sheet contains between 5% and 8% moisture. Forming a sheet of pulp material may include providing a pulp slurry to a headbox having a slice and carrying the pulp slurry that exits from the slice away from the headbox using, for example, a Fourdrinier. The Fourdrinier may also partially dry the sheet.

The sheet may be partially dried by passing the sheet between rolls of a wet press or by passing the sheet between cans of a drying stage that may be filled with steam. Drying the sheet after applying the crack-reducing agent may include passing the sheet between cans of a drying stage where the cans may be filled with steam.

Applying a crack-reducing agent to surfaces of the partially dried sheet may include applying the crack-reducing agent to a roll that contacts a first surface of the sheet where the roll may rotate in a tray containing the crack-reducing agent or, alternatively, the crack reducing agent may be sprayed onto the roll. An applicator having holes through which the crack-reducing agent pours onto a second surface of the sheet may also be used. The crack-reducing agent may be applied using a size press and/or may be sprayed directly onto surfaces of the sheet. A wet calendar stack may be used to apply an additional amount of the crack-reducing agent to the paper.

## BRIEF DESCRIPTION OF DRAWINGS

FIG. 1 is a schematic diagram illustrating a paper making process according to the invention.

FIGS. 2A and 2B illustrate a size press used to apply a polymer emulsion according to the present invention.

FIG. 3 is a schematic diagram of a wet calendar stack according to the present invention.

FIG. 4 is a schematic diagram of a size press in an alternative embodiment according to the present invention.

FIG. 5 is a schematic diagram of a size in an alternative embodiment according to the present invention.

## DETAILED DESCRIPTION OF THE PREFERRED EMBODIMENTS

Referring to FIG. 1, a schematic diagram 10 illustrates operation of a conventional Fourdrinier paper making machine that is modified and enhanced in a manner

described in detail below. Note that although the invention is illustrated herein using a Fourdrinier paper making machine, it will be appreciated by one of ordinary skill in the art that it would be straight-forward to adapt the invention to other types of paper making machines.

The paper making machine provides a continuous sheet of paper **12** as an output. The sheet **12** may be rolled up at the output by conventional means (not shown) and then subsequently used to make corrugating medium in a conventional manner, such as by using a conventional corrugator to form flutes in the sheet **12**.

A headbox **14** is provided with a pulp slurry containing any one of a variety of conventional combinations of hardwood pulp, softwood pulp, kraft pulp, sulfite soda pulp, ground wood, semi-ground wood, and/or semi-chemical or recycled pulp mixed with water and perhaps other conventional and well-known components that facilitate the paper making process. The specific combination of elements selected for the pulp slurry depends on a variety of functional factors familiar to one of ordinary skill in the art.

The pulp slurry exits from the headbox **14** via a slice **16** (a slit in the bottom front portion of the headbox **14**). The pulp slurry thus forms a sheet of pulp onto a conventional Fourdrinier **18** which continuously turns in the direction illustrated by arrows shown thereon in order to carry the output from the slice **16** away from the headbox **14**. The Fourdrinier **18** includes a wire mesh conveyor belt **19** that allows moisture from the sheet **12** to gravity drain, thus partially drying the sheet **12**. A vacuum can also be applied underneath the wire mesh conveyor belt **19** to facilitate additional drying.

Following the conveyor belt **18** is a wet press section **20** which, in the embodiment illustrated herein, consists of six rolls **22–27** forming three presses. The wet press section **20** removes additional moisture from the sheet **12** by applying pressure thereto. The rolls **22, 23** cooperate to press liquid out of the sheet **12**. Similarly, the rolls **24, 25** and the rolls **26, 27** cooperate to press additional moisture out of the sheet **12**.

Following the wet press section **20** is a first drying stage **30** which includes a plurality of dryer cans **32–39**. The dryer cans **32–39** are implemented in a conventional manner using hollow cylinders that may be filled with steam to heat the dryer cans **32–39**. The sheet **12** winds around the dryer cans **32–39** as shown in FIG. 1 and is heated in order to remove additional moisture therefrom.

After the first drying stage **30**, the sheet **12** is in a partially dry state. The partially dry sheet **12** may contain between 1% and 25% (by weight) of moisture. In a preferred embodiment, the partially dry sheet **12** contains between 5% and 8% moisture. Having the sheet **12** be partially dry facilitates the sheet **12** acquiring additional additives, as set forth in more detail below. However, if the amount of moisture contained in the partially dry sheet **12** is allowed to be too high, the sheet **12** will not have enough strength to withstand follow-on processing.

Following the first drying stage **30** is a size press **40** which includes a pair of rolls **42, 43**, a tray **45** and an applicator **46**. The partially dry sheet **12** passes between the rolls **42, 43** of the size press **40**. The roll orientation is the angle of a tangent line formed at the point of contact of the rolls **42, 43**. Other size presses having relative roll orientations different than that illustrated herein for the size press **40** may also be used.

The tray **45** contains a crack-reducing agent **48** that is applied to the lower surface of the sheet **12** by the roll **42**.

The roll **42** rotates through the crack-reducing agent **48** in the tray **45** and thus, as the sheet **12** moves through the size press **40**, the crack-reducing agent **48** is transferred onto the lower surface of the sheet **12** by the roll **42**. The applicator **46** also contains the crack-reducing agent **48**. The applicator **46** pours the crack-reducing agent **48** onto the top portion of the sheet **12**. The roll **43** then spreads the crack-reducing agent on the top portion of the sheet **12**. Thus, the combination of the tray **45**, the rolls **42, 43**, and the applicator **46** apply the crack-reducing agent **48** to both surfaces of the sheet **12**. Having the sheet **12** be partially dry prior to reaching the size press **40** facilitates absorption of the crack-reducing agent **48** by the sheet **12**. If the sheet were completely dry upon reaching the size press **40**, the crack-reducing agent **48** would not be absorbed as efficiently.

Following the size press **40** is a second drying stage **50** that includes a plurality of dryer cans **52–59**. Operation of the second drying stage **50** is similar to operation of the first drying stage **30**, described above, except that the drying stage **50** dries both the sheet **12** and dries the crack-reducing agent **48** that has been applied to the sheet **12** at the size press **40**. In another embodiment different than that illustrated in FIG. 1, the first drying stage **30** has eighteen dryer cans and the second drying stage **50** has eight dryer cans.

Referring to FIG. 2A, the size press **40** is illustrated in greater detail. The sheet **12** passes between the rolls **42, 43**. The applicator **46** applies the crack-reducing agent **48** to the upper surface of the sheet **12** while the roll **42** applies the crack-reducing agent **48** to the lower surface of the sheet **12**. The crack-reducing agent **48** that is applied to the upper surface of the sheet **12** is spread onto the upper surface of the sheet **12** by the roll **43**. Any excess crack-reducing agent **48** that is not taken up by the sheet **12** after passing through the rolls **42, 43** drips back into the tray **45**.

Referring to FIG. 2B, a schematic top view of the size press **40** illustrates application of the crack-reducing agent **48** to the upper surface of the sheet **12**. The applicator **46** includes a pipe-like portion having holes in the underside thereof. The crack-reducing agent **48** pours through the holes in the pipe of the applicator **46** onto the sheet **12**. The crack-reducing agent **48** that is thus applied to the upper surface of the sheet **12** is subsequently spread onto the upper surface of the sheet **12** by the roll **43**.

Referring to FIG. 3, a wet calendar stack **60** is optionally provided following the second drying stage **50**. The wet calendar stack **60** includes a plurality of rolls **62–66** through which the sheet **12** is threaded in a serpentine fashion. The wet calendar stack **60** also includes a high-water box **68** and a low-water box **70**, both of which contain the crack-reducing agent **48** (or perhaps a different crack-reducing agent than that applied at the size press **40**). The high-water box **68** provides the crack-reducing agent **48** to a first surface of the sheet **12** by first applying the crack-reducing agent **48** to the roll **63** which then contacts the first surface of the sheet **12**. Similarly, the low-water box **70** applies the crack-reducing agent **48** to a second surface of the sheet **12** by first applying the crack-reducing agent **48** to the roll **64** which contacts the second surface of the sheet **12**. Optionally, the wet calendar stack **60** can be followed by one or more additional wet calendar stacks (not shown) and/or by one or more dry calendar stacks (not shown) that do not apply a crack-reducing agent to the sheet **12**. The additional wet calendar stacks may apply the crack-reducing agent **48** and/or other additives to the sheet **12**. In another embodiment not illustrated in FIG. 3, a wet calendar stack having six rolls followed by a dry calendar stack having eight rolls are used together. Applying additional amounts of the crack-

reducing agent **48** using the wet calendar stack **60** allows the crack-reducing agent **48** to be applied in layers, thus facilitating a more even and perhaps thicker coating.

In a preferred embodiment, the crack-reducing agent **48** is manufactured using the following steps:

1. Place 900 gallons of water at ambient temperature into a mixing tank.
2. Add 250 milliliters of a defoamer such as Hercules Advantage 831 manufactured by Hercules Incorporated of Wilmington, Del.
3. Add 470 wet pounds of oxidized polyethylene wax emulsion such as ECC-3060 manufactured by the Eldorado Chemical Company, Inc. of San Antonio, Tex.
4. Add additional water so that the total volume in the mixing tank is 1,000 gallons.
5. Agitate the solution for five minutes to mix well.

The crack-reducing agent **48** is specifically formulated to reduce cracks when the paper is subsequently corrugated and may be manufactured via a plurality of alternative means. Alternative crack-reducing agents may comprise aqueous dispersions of metallic soaps, high solid lubricant blends containing calcium stearate soy-lecithin/oleic acid blends and mineral oil/sulfated petroleum oil blends. In addition, the waxes may be paraffin microcrystalline or oxidized polyethylene having either a high or a low density. The wax emulsion may be diluted with water in ratios between 0.25 and 20 percent.

Referring to FIG. 4, an alternative size press **40'** having rolls **42'**, **43'** is shown. In the embodiment shown in FIG. 4, the crack-reducing agent **48** is applied directly to the roll **42'** via a sprayer **72** while the crack-reducing agent **48** is applied directly to the roll **43'** via a sprayer **73**. The crack-reducing agent **48** thus sprayed onto the rolls **42'**, **43'** is applied to surfaces of the sheet **12** by the rotating action of the rolls **42'**, **43'**.

Referring to FIG. 5, an alternative size press **40"** uses two rolls **42", 43"**. The crack-reducing agent **48** is applied to the lower surface of the sheet **12** via a sprayer **82** and to the upper surface of the sheet **12** via a sprayer **83**. The sprayers **82, 83** cooperate to provide the crack-reducing agent **48** simultaneously to both surfaces of the sheet **12**. The applied crack-reducing agent **48** is subsequently spread onto the sheet **12** by the rolls **42", 43"**.

While the invention has been disclosed in connection with the preferred embodiments shown and described in detail, various modifications and improvements thereon will become readily apparent to those skilled in the art. Accordingly, the spirit and scope of the present invention is to be limited only by the following claims.

What is claimed is:

1. A method of making paper for corrugating medium, comprising the steps of:
  - (a) forming a sheet of pulp material;
  - (b) partially drying the sheet of pulp material to provide a partially dried sheet;
  - (c) applying an effective amount of a crack-reducing agent to surfaces of the partially dried sheet, the crack-reducing agent being absorbed in the partially dry sheet, wherein the crack-reducing agent comprises a pigment-free polyethylene wax emulsion diluted with water in ratios between 0.25 and 20 percent, and wherein the crack-reducing agent is applied using a size press; and

(d) drying the partially dried sheet after applying the crack-reducing agent to provide a sheet of paper for corrugating medium, whereby absorption of the crack-reducing agent inhibits formation of cracks when the paper is corrugated.

2. A method of making paper for corrugating medium, according to claim 1, wherein the partially dry sheet contains between 1% and 25% by weight of moisture.

3. A method of making paper for corrugating medium, according to claim 2, wherein the partially dry sheet contains between 5% and 8% by weight of moisture.

4. A method of making paper for corrugating medium, according to claim 1, wherein forming a sheet of pulp material comprises:

- (e) providing a pulp slurry to a headbox having a slice; and
- (f) carrying the pulp slurry that exits from the slice away from the headbox.

5. A method of making paper for corrugating medium, according to claim 4, wherein the pulp slurry that exits from the slice is carried away by a Fourdrinier.

6. A method of making paper for corrugating medium, according to claim 1, wherein partially drying the sheet includes passing the sheet between rolls of a wet press.

7. A method of making paper for corrugating medium, according to claim 6, wherein partially drying the sheet further includes passing the sheet between cans of a drying stage.

8. A method of making paper for corrugating medium, according to claim 7, wherein the cans of the drying stage are filled with steam.

9. A method of making paper for corrugating medium, according to claim 1, wherein partially drying the sheet includes passing the sheet between cans of a drying stage.

10. A method of making paper for corrugating medium, according to claim 9, wherein the cans of the drying stage are filled with steam.

11. A method of making paper for corrugating medium, according to claim 1, wherein applying a crack-reducing agent to surfaces of the partially dried sheet includes applying the crack-reducing agent to a roll that contacts a first surface of the sheet.

12. A method of making paper for corrugating medium, according to claim 11, wherein applying the crack-reducing agent to a roll includes providing the crack-reducing agent in a tray through which the roll rotates.

13. A method of making paper for corrugating medium, according to claim 11, wherein applying the crack-reducing agent to a roll includes spraying the crack-reducing agent onto the roll.

14. A method of making paper for corrugating medium, according to claim 11, wherein applying the crack-reducing agent to surfaces of the partially dried sheet includes applying the crack-reducing agent to a second surface of the sheet using an applicator having holes therein through which the crack-reducing agent pours onto the second surface.

15. A method of making paper for corrugating medium, according to claim 1, further comprising the step of:

using a wet calendar stack to apply an additional amount of the crack-reducing agent to the paper.